

Nov. 12, 1940.

A. C. ESTEP

2,221,130

METHOD OF MAKING INGOT MOLD PLUGS

Original Filed Sept. 3, 1937



BY

ARTHUR C. ESTEP  
Ridley & Watt,  
ATTORNEYS.

INVENTOR.

## UNITED STATES PATENT OFFICE

2,221,130

## METHOD OF MAKING INGOT MOLD PLUGS

Arthur C. Estep, Waynesburg, Ohio, assignor to  
The Whitacre-Greer Fireproofing Company,  
Waynesburg, Ohio, a corporation of Ohio

Original application September 3, 1937, Serial No.  
162,315. Renewed May 25, 1939. Divided and  
this application June 24, 1939, Serial No. 281,002.

3 Claims. (Cl. 22—193)

- This invention relates to a method of making ingot mold plugs and more particularly to a ceramic or a refractory ingot mold plug particularly adapted for advantageous use with a "big-end-up" ingot mold. The instant application constitutes a division of my prior Patent No. 2,170,555 filed September 3, 1937, allowed June 9, 1938, and renewed May 25, 1939, renewal Serial No. 162,315.
- 10 In the art of casting ingots there has been a general adoption of the "big-end-up" type of ingot mold; that is, a mold having an open top with side walls gradually diverging from the bottom toward the top. A tapered hole is provided at the bottom of the mold which is closed by a sealing plug while the ingot is poured and the ingot, after cooling, is forced upwardly out of the mold. Prior to pouring the ingot the plug referred to is forced into the hole at the bottom of the mold which hole is tapered according to the accepted practice so that the plug may be driven into the hole and have a snug fit which prevents the escape of molten metal during the pouring of the ingot. Because of its ability to accommodate itself to the contour of the hole at the base of the ingot mold as by limited surface crushing or abrasion against the wall of the hole, an ingot mold plug formed of burned clay is capable of effecting an efficient seal. The present invention relates principally to the method of making refractory ingot mold plugs, the latter being particularly described and claimed in my aforesaid co-pending application.
- It is among the objects of my invention to provide a burned clay ingot mold plug and method of making the same whereby the plug will withstand the shock to which it may be subjected while being driven into the tapered hole of the ingot mold and will withstand the thermal and physical shock occasioned by the flow of molten metal into the mold. Another object is to provide a refractory plug which will not spawl in the area of contact with molten steel or otherwise give off non-metallics to the ingot. It is a further object of my invention to provide a method of making an ingot mold plug which will give in the finished plug certain structural characteristics of yielding strength whereby to resist deleterious fracture or spawling in use. It is also an object of my invention to provide an ingot mold plug with circular concentric laminations which will tend to restrict any fracture of the plug to the direction defined by the laminations. It is a further object of my invention to provide a method of making an ingot mold plug in which an

extruded clay tile cylinder is upset to form a plug having a truncated cone shape. It is a further object of my invention to provide a burned clay mold plug characterized by smooth troweled outer surfaces especially resistant to spawling and cracking. It is also among the objects of my invention to provide a method for making a mold plug in accordance with the preceding object. Further objects and advantages relating to economies of manufacture and characteristics of the finished mold plug will appear from the following description and the appended drawing in which—

Figure 1 is a view of a clay extrusion apparatus suited to extrude laminated cylindrical stock employed in my invention;

Figure 2 is a sectional view with parts broken away of an upsetting or molding apparatus made according to my invention;

Figure 3 is an enlarged sectional view of the relief mechanism employed in the upsetting or molding apparatus;

Figure 4 is a transverse sectional view (taken along the line 4—4 of Figure 5) of a mold plug constructed according to my invention;

Figure 5 is a plan view of the mold plug;

Figure 6 is a partial sectional showing of a mold plug according to my invention arranged within an ingot mold.

The first step in forming a mold plug corresponding generally to the objects outlined above comprises extruding wet clay stock of round cross section such as 4 in Figure 1. Preferably the clay stock is extruded from an auger machine 5 of the type in which the mass of wet clay being extruded is open to the atmosphere through a hopper as at 8 to facilitate the formation of laminations in the extruded stock 4. There is a tendency for extruded clay products to form laminations generally parallel to the walls of the extrusion die and in forming certain articles it is conventional practice to extrude from a chamber maintained at less than atmosphere pressure to prevent the formation of laminations. According to my invention, however, I prefer to take advantage of the laminating tendency referred to and therefore prefer that there be little or no deaerating of the extruded mass. In addition to insuring against deaerating the mix should be sufficiently "short" so that marked circular concentric laminations coaxial of the stock will be formed in portion 4. The clay may be fed to the auger machine 5 from a pug mill 7 in the usual manner and forced by an auger through the forming throat 13 and extrusion die 12. The extruded stock 4 is severed by wire cutters or

other suitable means into short cylindrical slugs 6 having a volume corresponding substantially to the volume of a finished mold plug.

Subsequent to the extrusion of the clay stock 4 and the cutting thereof to provide cylindrical slugs 6, the slugs are each transferred while in a plastic condition to an upsetting apparatus arranged to upset the cylindrical slug into a plug having a truncated cone shape. In Figure 2 I have illustrated a preferred form of upsetting apparatus in which a pair of cylindrical bores 19 and 20 are joined to each other by a tapered wall portion 21 which corresponds substantially to the shape of the finished mold plug. A back-up or ejector plunger 24 is positioned within the bore 19 to close the lower end of the upsetting chamber and the upsetting plunger 26 is arranged within the bore 20 so that it may be moved to close the opposite side of the mold plug chamber. I have shown in the dotted lines of Figure 2 a cylindrical mold plug blank 6 as positioned prior to its upsetting and the upset mold plug 30 resulting from the movement of the plunger 26 to its position shown fills the mold plug chamber.

I have found that by upsetting a cylindrical clay slug as above described that the exterior surface of the article is improved by the formation of a hard, tough spawl-resistant cover. The pressure upon the wet clay slug appears to bring moisture to the outer surface of the upset article and upon burning a thin cover or skin is formed which is resistant to spawling. The spawl resistant covering resulting from upsetting the slug as above described may be further improved by effecting a troweling action upon the outer surface of the slug during and/or after the upsetting. The troweling or wiping of the outer surface is preferably accomplished by rotating the plunger 26 and such rotation is preferably effected so as to effect no disturbance of the laminated structure within the body of the plug. The rotation of the plunger 26 may be accomplished by having the plunger shaft splined axially as at 43 so that the shaft may reciprocate within an internally splined worm gear 41 supported by a bracket 40. A spur gear 42 is arranged to mesh with and drive the worm gear 41. The rotation of the plunger 26 during and/or after the upsetting of the slug appears to effect a troweling of the surface which forces water and minute clay particles to the outer surface of the plug. Upon burning the smooth troweled outer surface of the plug acquires a hard, tough, skin-like cover which is resistant to spawling and thus contributes to the prevention of non-metallics being carried up into the ingot during the pouring thereof.

Due to the fact that as a practical matter in commercial production it is difficult or impossible to obtain a series of cylindrical slugs 6 which are of exactly the same volume and due to the fact that such plastic slugs are more or less incompressible, it would, in the absence of an apparatus such as I have provided, be difficult to obtain mold plugs completely shaped and filled. Because of the variation in volume of the cylindrical slugs and because it is desired to produce truncated cone shaped mold plugs of uniform height and full body, I have provided an upsetting apparatus which will compensate for the normal variations in the volume of the cylindrical slugs.

Preferably the back-up or ejector plunger 24 is

centrally apertured as at 25 (Figure 3) and carries in said aperture a piercing tool 27 which is normally urged upwardly to the limit of a slot such as 28 by a spring 29. Each of the cylindrical slugs 6 is initially cut so as to provide a volume of material less than the volume of the space between the two plungers 24 and 26. When the plastic slug 6 is forced downwardly into the upsetting chamber defined by the two plungers and the tapered wall 21, it will be observed that the piercing tool 27 is forced into the plastic mass and that the plastic slug offers a resistance to the movement of the plunger 26 until it has reached the end of the cylindrical bore 20 as shown. As the plunger 26 approaches the position shown it will be understood that the hydrostatic pressure in the slug being upset will force the piercing tool 27 downwardly out of the upsetting chamber against the resistance of the spring 29. The distance which the piercing tool is forced downwardly out of the upsetting chamber by the hydrostatic pressure in the plastic slug will depend upon the difference in volume between the cylindrical slug and the volume defined by the tapered wall 21 and the plungers 24 and 26 in their positions shown in Figure 2. It is possible according to the known methods of cutting plastic clay stock to cut cylindrical slugs in which the volumes will not vary with respect to each other more than the volume of the piercing tool 27 in its raised position. Thus it is possible with the usual known methods of wire cutting wet clay stock and the method and apparatus I have provided for upsetting such stock to obtain mold plugs having a truncated cone shape and having a uniform height and otherwise being uniform in their external dimensions.

The steps which include the cutting and upsetting of the plastic clay blank are preferably carried out in a manner which will not appreciably disturb the cylindrical laminations in the slug so that the finished upset plug will in effect comprise a series of tapered tubes more or less distinguishable from each other by laminations such as 16 shown in Figure 4. Subsequent to the upsetting as described in connection with Figures 2 and 3 the plastic mold plug is burned in the conventional manner and the resulting laminated upset and burned plug 32 is shown in Figures 4 and 5.

The finished plug may be inserted through the open end of an ingot mold 35 and driven into the base of the ingot mold to close the opening 36 therein as shown in Figure 6. Ordinarily an ingot mold plug of this type is forcibly wedged into the opening 36 by driving and jarring operations effected with a heavy timber or the like reciprocated from the open end of the ingot mold. The impact at the upper surface of the plug may be sufficient to effect a slight abrasion or surface fracture of the conical walls of the ceramic mold plug so that the plug will acquire substantially the shape of the aperture 26 to which it is fitted and form a tight seal against the molten metal poured into the mold.

It will be observed that even though the impact of a heavy timber such as is required to force the plug into the mold opening 26 be such as would break or fracture the plug, the truncated laminations defined by surfaces 16 tend to permit the plug sections between said surface to "slip" with respect to each other. It is possible that a mold plug of my invention could be

driven into the opening 36 with such force that the plug is fractured two or three times on different concentric conical surfaces 16 and yet its utility as a mold plug will be preserved. It will 5 also be understood that such plug fracture caused by internal stresses within the plug growing out of the burning and shrinkage will be more or less confined to the surfaces 16 and that regardless of the cause of plug fracture the usefulness 10 of the plug is not destroyed as long as the fracture is restricted to concentric surfaces such as 16. Among the desirable characteristics of a burned clay mold plug is the resistance of the plug to spawling at the surface due to the thermal 15 shock caused by the inflowing molten metal as the mold is being poured. A resistance to spawling or surface fracture is desired in that there is a tendency for the molten metal to float broken or spawled particles of the plug and carry 20 the same up into the ingot. An ingot carrying particles of non-metallic is obviously defective for rolling purposes. It will be observed that due to the laminations or curved fracture surfaces such as 16 the thermal expansion caused by the 25 sudden inflow of molten metal is broken up or limited in its action by the fracture surfaces 16. The surfaces 16 appear to prevent a heat flow across the upper surface of the plug such as would be sufficient to break away the top layer 30 of the plug from the body of the plug. While it is difficult to determine all of the reasons why a mold plug having concentric laminations is especially resistant to spawling or surface fracture during the pouring of the ingot I have found 35 that mold plugs having such laminations do resist surface spawling to a marked degree.

Although I have illustrated and described certain specific forms in which my invention may

be practiced, various changes and modifications will occur to those skilled in the art, all within the precepts of my invention, and I do not care to be limited to the precise embodiments herein particularly described or in any manner other than by the claims appended hereto when construed with the range of equivalents to which I may be entitled in view of the prior art.

I claim:

1. That method of making an ingot mold plug 10 which comprises extruding a length of clay stock with laminations extending axially of the stock, cutting cylindrical blanks from said lengths of stock having a volume corresponding substantially to the volume of the finished mold plug and 15 upsetting said blanks in a direction parallel to the axis of the stock to form a truncated cone plug, troweling the outer surface of said plug during and/or subsequent to the upsetting thereof without appreciably disturbing the said laminations and thereafter burning the shaped plug in a kiln.

2. That method of making an ingot mold plug which comprises extruding clay stock, cutting said stock transversely to produce blanks proportioned to form a mold plug, upsetting said blanks 25 into conically surfaced plugs by compressing said blanks in the direction of extrusion and burning said plugs.

3. That method of making an ingot mold plug 30 which comprises extruding a length of clay stock with laminations extending axially thereof, cutting said stock transversely to produce cylindrical blanks proportioned to form a mold plug, upsetting said blanks into conical plugs by compressing 35 said plugs in a direction parallel to the axis of the stock.

ARTHUR C. ESTEP.